

## UNITED STATES PATENT OFFICE

2,284,241

## CORROSION INHIBITION

James H. Werntz, Wilmington, Del., assignor to  
 E. I. du Pont de Nemours & Company, Wil-  
 mington, Del., a corporation of Delaware

No Drawing. Application May 13, 1939, Serial  
 No. 273,426

15 Claims. (Cl. 106—14)

This invention relates to inhibiting the corrosion of metals and particularly to inhibiting rust formation on ferrous metals due to the effect of moisture and oxygen.

It is well known that the surfaces of metals, and particularly the surfaces of ferrous metals, normally tend to corrode with the formation of rust when subjected to the effect of moisture and oxygen. Many methods have been proposed for preventing or inhibiting such corrosion and rust formation. One of the commonest methods proposed has comprised coating the metallic surfaces with a thin film of an oily material such as lanolin, Vaseline, and similar materials. While such oily materials are to some extent effective, they have not proved to be entirely satisfactory in practice.

It is frequently desirable to apply to metal surfaces, and particularly to ferrous metal surfaces including tin-plate, lithographic inks, paints, lacquers and the like. When the metal surfaces are preserved with oily materials, it is generally necessary to remove such oily materials from the metallic surfaces prior to the application of lithographic inks, paints, lacquers and the like, as such oily materials greatly decrease the receptivity of the metal surface for inks, paints, lacquers and the like, and also decreases the retention of the inks, etc., on the metallic surfaces. This effect of the oily materials frequently goes so far as to prevent any application of the inks, etc., to the metal surface bearing the oily materials. When such oily materials are removed from the metal surfaces, the protective effect of the oily materials is lost. Also, removal of the oily materials from the metallic surfaces involves an additional step requiring labor and expense.

It is a primary object of this invention to provide materials for coating metallic surfaces, particularly the surfaces of ferrous metals, which materials will be more effective for retarding corrosion and the formation of rust and at the same time will not decrease the receptivity of the metallic surfaces for lithographic inks, paints, lacquers and the like, or decrease the retentivity of such inks, etc., by the metallic surfaces. Another object is to provide a method for treating metallic surfaces such as the surfaces of ferrous metals to inhibit corrosion of, and rust formation on, such metallic surfaces. A further object is to provide metals and particularly ferrous metals, the surfaces of which will have a lesser tendency to be corroded and rusted, and which at the same time will have a high receptivity for, and retentivity of, lithographic inks, paints, lacquers and the like. Still further objects are to provide new compositions of matter and new articles of manufacture, and to advance the art. Still other objects will appear hereinafter.

The above and other objects may be accomplished in accordance with my invention, which comprises coating the surfaces of metals, and particularly the surfaces of ferrous metals, with a thin film of a composition containing an acyclic aliphatic acid-ester of a polycarboxylic acid, the acyclic aliphatic radical containing at least 6 carbon atoms and preferably long chains of from about 8 to about 18 carbon atoms. These acid-esters may be otherwise designated as those derived from a polycarboxylic acid and an acyclic aliphatic alcohol containing at least 6 carbon atoms. While it is preferred to employ the alkyl esters of the polycarboxylic acids, and particularly the esters which consist of the elements carbon, hydrogen and oxygen, either or both the aliphatic radical and the acid radical may contain substituents such as halogen, hydroxy, nitro, alkoxy, carboxyl or ester groups, as well as alkyl groups. Preferably, the acid is a dicarboxylic acid in which the two carboxyl groups are separated by at least two intervening carbon atoms. While the acids may be either aliphatic or aromatic, the aromatic acids are preferred and of these, I particularly prefer phthalic acid and its homologs.

I have found that the acid esters of my invention, when applied to metallic surfaces, and particularly to the surfaces of ferrous metals, in the form of a thin film, are very effective for retarding corrosion, particularly the formation of rust, of the metallic surfaces caused by moisture and oxygen. When such acid-esters are used as the sole coating substance, or are used in combination with other substances which do not decrease the receptivity of the metal for lithographic inks, paints, lacquers and the like or the retention thereof by the metals, then the receptivity and retentivity of the metal surfaces are not deleteriously affected but are, in some cases such as when phthalates are used, improved. In other words, when the acid-esters of my invention, and particularly the phthalates, are employed in the absence of substances tending to reduce the receptivity of the metal surfaces for ink, lacquer, paint and the like, the metal surfaces can be lithographed, painted, lacquered or otherwise coated at least as successfully as they can be lithographed, etc. in the absence of a coating, without requiring removal of the acid-esters from the metallic surfaces prior to lithographing, painting, lacquering, and the like. The long chain acid phthalates, such as the "Lorol" acid phthalates and dodecyl acid phthalate, are particularly effective for this purpose and materially improve the receptivity of the metal surfaces for lithographic inks, paints, lacquers and the like.

In other cases, where it is not proposed to lithograph, paint, or otherwise coat the metallic surfaces or where it is desirable to improve the

corrosion protection at the sacrifice of paint and ink receptivity, the acid esters of my invention may be employed together with a non-volatile mineral, petroleum, vegetable or animal oil such as "Vaseline," "Nujol" and lanolin. When my compounds are employed with such oils, it will generally be most practical and convenient to incorporate them in the oil prior to application to the metal surface. The use of such oils with my compounds will increase the protection against corrosion and rust formation, particularly where severe moisture conditions or corrosive gases are encountered. However, such oils will naturally be expected to decrease to a large extent the beneficial effects of my compounds on the receptivity and retentivity of the metallic surfaces for lithographic inks, paints, lacquers, and the like.

Although these compounds will usually be applied to metal surfaces by means of a solution using such well known processes as dipping, spraying, wiping and brushing, it will be desirable at times to use other methods of application. A material which melts at reasonably low temperatures and which undergoes no decomposition in the region of its melting point, may be applied in the liquid form without a diluent of any kind, but the application of the material should be regulated so that the final protective film conforms to the thickness limits found suitable for these compounds. When in solid form, these compounds may also be applied to the metal surface in a finely divided condition, the protective layer being formed by fusing the solid particles to a continuous coating at a suitable temperature. The protective agent may also be emulsified or dispersed in a liquid which is not a true solvent and applied to the metal surface in this form with subsequent evaporation of the carrier. In certain cases it may be advantageous to provide metal articles with a protective surface layer by permitting the condensation of vapor from one of these compounds upon the metal surface.

When solvents are employed, they may be of any desired concentration. However, it will generally be undesirable to use solutions of more than 15% concentration. The preferred solutions for most purposes will usually have a concentration of from about 1% to about 8% of the acid-ester. The film of material will preferably be of such thickness as will be obtained by the coating of from 10,000 to 80,000 square feet of surface with one pound of ester or anti-corrodent composition. Solutions of 1 to 8% concentration will generally provide such thickness of film.

Amongst the compounds of my invention which are particularly desirable are:

Dodecyl acid phthalate  
\* "Lorol" acid phthalate  
Octadecenyl acid phthalate  
Castor oil acid phthalate  
Octadecyl acid phthalate  
Octadecyl acid maleate

\* Alcohol employed in making this compound was a mixture of normal primary monohydric aliphatic alcohols obtained by the carboxylic reduction of coconut oil. This mixture of alcohols is known to the trade as "Lorol" alcohol. The resulting product is a mixture of the acid phthalate esters of such alcohols.

In order to illustrate more clearly the preferred modes of carrying my invention into effect, the following examples are given:

### Example I

Cold rolled 20-gauge steel sheet is prepared for storage and shipment by cleaning in a vapor degreaser, immersing briefly in a 4% solution of dodecyl acid phthalate in toluol, draining and drying at room temperature.

### Example II

10 Cold reduced 24-gauge steel sheet is cleaned by scrubbing in an alkali silicate solution, rinsed with fresh water and dried in a current of hot air. The sheet, while still warm, is passed between cloth rolls saturated with a 3% solution of "Lorol" acid phthalate in xylol. The solvent evaporates readily during a short travel on belt conveyors and the sheets are then inspected and stacked for packaging. After six weeks' storage in an industrial atmosphere, exposed to average condensation conditions, untreated control sheets were badly rusted. Steel sheets coated with lanolin in this manner showed comparatively large rust spots uniformly distributed over each sheet. On the other hand, steel sheets treated as above were rust-free with the exception of very small rust spots scattered along the outer edges of the sheets.

### Example III

30 Iron wire is drawn in the usual manner and, after leaving the last die, the wire is passed between felt pads impregnated with octadecenyl acid phthalate. A treatment of this type does not affect the appearance of the wire, but will prevent rust formation over extended periods of storage.

### Example IV

40 Wire nails are fabricated and burnished in the usual manner, after which they are basket dipped in a solution comprising 2% octadecyl acid maleate and 10% light mineral oil in low flash naphtha. The nails are then drained and dried by tumbling in a current of warm air. Such products are especially suited for the export trade because of their resistance to corrosion induced by salt air.

45 In order to show further the effects of my compounds, and particularly in relation to some related compounds not within my invention, the results of a number of tests are given in the following tables, in which "control" refers to similar untreated steel panels subjected to the same conditions as the treated steel panels:

Table I

55 In the following tests, the anticorrosive agents were tested by applying them to sheet steel panels by dipping in a 4% toluene solution and, after removing the solvent by evaporation, subjecting the panels to 18 days' continuous water condensation.

| Agent                          | Comparative rating* | Observations on rusting             |
|--------------------------------|---------------------|-------------------------------------|
| "Vaseline".....                | 3                   | Heavy continuous rust.              |
| "Nujol".....                   | 3                   | Do.                                 |
| Control.....                   | 3                   | Do.                                 |
| Dodecyl acid phthalate.....    | 9                   | Very slight rust in isolated spots. |
| Didodecyl maleate.....         | 6                   | Large rust spots.                   |
| Distyryl maleate.....          | 3                   | Heavy continuous rust.              |
| Castor oil acid phthalate..... | 8                   | Slight scattered rust spots.        |

\* The rating as here given is an arbitrary figure which is based on the figure 10 for complete absence of rusting and 0 for complete rusting over the whole surface of the panel.

Table II

The following agents were applied on bright steel panels to a thickness of 0.1 mil by rubbing the agent on the steel. The treated panels were then exposed to outdoor weathering for a period of 18 days.

| Agent                         | Rating* | Observations on rusting           |
|-------------------------------|---------|-----------------------------------|
| "Nujol".....                  | 0       | Completely covered with rust.     |
| Control.....                  | 0       | Do.                               |
| Dodecyl acid phthalate.....   | 9       | Very slight scattered rust spots. |
| Octadecyl acid phthalate..... | 8       | Slight scattered rust spots.      |

\* See Table I for definition of "rating."

Table III

The following agents were applied on bright steel panels by dipping in a 2% toluene solution (except where otherwise indicated) and, after removal of the solvent by evaporation, exposing the panels to continuous water condensation for seven days:

| Agent                                                                                                              | Rating |
|--------------------------------------------------------------------------------------------------------------------|--------|
| None (control).....                                                                                                | 3 to 4 |
| "Vaseline".....                                                                                                    | 3      |
| Nonyl acid phthalate.....                                                                                          | 9      |
| Dodecyl acid phthalate.....                                                                                        | 9      |
| Castor oil acid phthalate.....                                                                                     | 9      |
| Cellulose acid phthalate (1/2% solution in toluene).....                                                           | 7      |
| Cyclohexyl butyl phthalate.....                                                                                    | 4      |
| Diethyl fumarate.....                                                                                              | 3      |
| Diethyl tartrate.....                                                                                              | 3      |
| Diethyl malonate.....                                                                                              | 3      |
| Diethyl citrate.....                                                                                               | 3      |
| Acid phthalate of the alcohols of seven and eight carbon atoms obtained by the hydrogenation of carbon oxides..... | 9      |
| Diisoamyl oxalate.....                                                                                             | 4      |
| Stearyl acid phthalate.....                                                                                        | 9      |

Results on the neutral esters are given for comparison.

Table IV

The following agents were applied in 4% toluene solutions to steel panels phosphatized by commonly known commercial processes, the solvent was allowed to evaporate, and the panels were then exposed to outdoor weathering for 19 days:

| Agent                       | Rating |
|-----------------------------|--------|
| None (control).....         | 1      |
| Lanolin.....                | 5      |
| Stearyl acid phthalate..... | 8      |

The examples and tests hereinbefore given merely illustrate the results obtained with some of the compounds of my invention. Other desirable compounds of my invention are:

"Lorol" acid nitrophthalate  
Octyl acid phthalate  
Cetyl acid phthalate  
Acid phthalates of alcohols from petroleum  
Cetyl acid citrate  
9,10-octadecenyl acid citrate  
Dodecyl acid succinate  
Dodecyl acid maleate  
"Lorol" acid maleate

The following alcohols and acids may be employed in preparing suitable compounds of my invention.

Alcohols

| Alcohols                                                                          | Acids                  |
|-----------------------------------------------------------------------------------|------------------------|
| Hexyl                                                                             | Succinic               |
| Decyl                                                                             | Monomethyl succinic    |
| Hexadecyl                                                                         | Dimethyl succinic      |
| Myrciel                                                                           | Trimethyl succinic     |
| Tetradecyl                                                                        | Phenyl succinic        |
| Dodecyl                                                                           | Maleic                 |
| Octadecyl                                                                         | Phenyl maleic          |
| Linoleyl                                                                          | Citric                 |
| Octyl                                                                             | Malic                  |
| Octadec-9-enyl                                                                    | Glutaric               |
| "Lorol"                                                                           | Adipic                 |
| ""Stenol"                                                                         | Suberic                |
| Cyclohexyl                                                                        | Fumaric                |
| Methylcyclohexyl                                                                  | Citra-conic            |
| Naphthetyl                                                                        | Citra-mallic           |
| Pentadecyl-8                                                                      | Iso-Phthalic           |
| Heptadecyl-7                                                                      | tere-Phthalic          |
| Tridecyl-6                                                                        | o-Carboxy cinnamic     |
| Alcohols of 6 or more carbon atoms obtained by the hydrogenation of carbon oxides | o-Carboxyhydrocinnamic |
| Homologs and isomers of above                                                     | Uvitic                 |

\*\* "Stenol" is a mixture of alcohols obtained by the catalytic reduction of the fatty acids from sperm oil.

Still other compounds within my invention may be obtained from alcohols obtained by the oxidation of petroleum, or by the reduction of the acids obtained from petroleum or from the oxidation of petroleum. Further, mixtures of two or more of the above esters, mixtures obtained by reacting any one of the acids with a

25 mixture of any of the above alcohols and mixtures obtained by reacting any one of the above alcohols with a mixture of two or more of the above acids may be employed.

30 My compounds may be used for the temporary protection of metal which is to be fabricated further, such as steel sheet, wire and tubing, or may be used in treating finished articles such as machine parts, tools, guns, locks, and the like. These compounds are also particularly well 35 adapted to the protection of ferrous metal articles such as bolts, nuts, nails, bearings, cutlery, gears, metallic cases, and the like. They may also be used for the treatment of ferrous metal articles which have been provided with a surface 40 coating of some other mineral or alloy such as chromium, copper, nickel, cadmium, zinc, brass, aluminum, tin, lead, etc. In addition, these compounds may be applied to the surfaces of other metals and alloys, particularly those used for structural shapes and articles of commerce.

45 Among such metals are zinc, brass, bronze, aluminum, tin, copper, pewter, lead, magnesium, cadmium, nickel, duralumin, and the like.

50 My compounds are definitely more effective in inhibiting corrosion due to moisture condensation than equivalent amounts of such commonly used materials as wool fat and mineral oil. The principal advantage of my compounds over the former type of compound is realized when the treated metal surface is to be painted or lithographed subsequently. Neither wool fat nor mineral oil can be tolerated on a metal surface which is being lithographed, painted or lacquered, while my compounds, and particularly the "Lorol" acid

55 phthalate and dodecyl acid phthalate, actually improve the ink and paint receptivity of the metal surface and promote the flow and leveling of the applied ink, paint, lacquer or the like. Thus, instead of necessitating an expensive degreasing operation as is generally necessary with the here-

60 tofore proposed oily materials, the protection of the metal surfaces with the compounds of my invention produces a better lithographing and painting base and is of material assistance in the 65 finishing operations on many manufactured ar-

70

ticles without requiring the use of a degreasing or equivalent operation.

While I have disclosed the preferred embodiments of my invention and the preferred modes of carrying the same into effect, it will be readily apparent to those skilled in the art that many variations and modifications may be made therein without departing from the spirit of my invention. Accordingly, the scope of my invention is not to be limited by the specific embodiments specifically illustrated in the body of this specification, but the true scope of my invention is as defined in the appended claims.

I claim:

1. A ferrous metal having its surface coated with a thin film consisting of an aliphatic acid-ester of a polycarboxylic acid, in which the aliphatic radical is a member of the group consisting of acyclic aliphatic, cyclohexyl and naphthenyl radicals and contains at least 6 carbon atoms, said ester consisting of the elements carbon, hydrogen and oxygen.

2. A ferrous metal having its surface coated with a thin film consisting of an acyclic aliphatic acid-ester of a dicarboxylic acid in which the carboxyl groups are separated by at least 2 intervening carbon atoms, the acyclic aliphatic radical containing at least 6 carbon atoms, said ester consisting of the elements carbon, hydrogen and oxygen.

3. A ferrous metal having its surface coated with a thin film consisting of an acyclic alkyl acid-ester of a dicarboxylic acid in which the carboxyl groups are separated by at least 2 intervening carbon atoms, the acyclic alkyl radical containing at least 8 carbon atoms, said ester consisting of the elements carbon, hydrogen and oxygen.

4. A ferrous metal having its surface coated with a thin film consisting of an acyclic aliphatic acid-ester of a phthalic acid in which the acyclic aliphatic radical contains at least 6 carbon atoms, said ester consisting of the elements carbon, hydrogen and oxygen.

5. A ferrous metal having its surface coated with a thin film consisting of an acyclic alkyl acid-ester of phthalic acid in which the acyclic alkyl radical contains at least 6 carbon atoms.

6. A rust-proofing composition for metals consisting of a solution, in an inert volatile solvent, of an aliphatic acid-ester of a polycarboxylic acid, in which the aliphatic radical is a member

of the group consisting of acyclic aliphatic, cyclohexyl and naphthenyl radicals and contains at least 6 carbon atoms, said ester consisting of the elements carbon, hydrogen and oxygen.

5 7. A rust-proofing composition for metals consisting of a solution, in an inert volatile solvent, of an acyclic alkyl acid-ester of a dicarboxylic acid in which the carboxyl groups are separated by at least 2 intervening carbon atoms, the acyclic alkyl radical containing at least 8 carbon atoms, said ester consisting of the elements carbon, hydrogen and oxygen.

10 8. A rust-proofing composition for metals consisting of a solution, in an inert volatile solvent, of an acyclic alkyl acid-ester of a phthalic acid in which the acyclic alkyl radical contains at least 6 carbon atoms, said ester consisting of the elements carbon, hydrogen and oxygen.

15 9. A rust-proofing composition for metals consisting of a solution, in an inert volatile solvent, of an acyclic aliphatic acid-ester of phthalic acid in which the acyclic aliphatic radical contains at least 6 carbon atoms, said ester consisting of the elements carbon, hydrogen and oxygen.

20 10. A ferrous metal having its surface coated with a thin film consisting of the acid phthalates of the mixture of normal primary monohydric aliphatic alcohols obtained by the carboxylic reduction of coconut oil.

25 30 11. A rust-proofing composition for metals consisting of a solution, in an inert volatile solvent, of the acid phthalates of the mixture of normal primary monohydric aliphatic alcohols obtained by the carboxylic reduction of coconut oil.

35 12. A ferrous metal having its surface coated with a thin film consisting of the acid maleates of the mixture of normal primary monohydric aliphatic alcohols obtained by the carboxylic reduction of coconut oil.

13. A ferrous metal having its surface coated with a thin film consisting of stearyl acid phthalate.

40 14. A rust-proofing composition for metals consisting of a solution, in an inert volatile solvent, of the acid maleates of the mixture of normal primary monohydric aliphatic alcohols obtained by the carboxylic reduction of coconut oil.

45 15. A rust-proofing composition for metals consisting of a solution, in an inert volatile solvent, of stearyl acid phthalate.

JAMES H. WERNITZ.